

## UNITED STATES PATENT OFFICE

2,077,794

## REFRACTORIES

Frederic A. Harvey and Raymond E. Birch, Pittsburgh, Pa., assignors to Harbison-Walker Refractories Company, Pittsburgh, Pa., a corporation of Pennsylvania

No Drawing. Application June 4, 1935,  
Serial No. 24,988

## 5 Claims. (Cl. 106—9)

This invention relates to refractories, more particularly to chrome ore refractories.

It is among the objects of the invention to provide chrome ore refractories possessing improved characteristics, particularly with regard to strength and weight, as compared with those manufactured heretofore, which exhibit relatively low shrinkage upon burning and reheating, in which desirable characteristics of chrome ore refractories, such as resistance to acid and basic conditions, and relatively low porosity, are retained wholly or in such large part as not to reduce their desirability, and which are relatively cheap and readily made.

15 Chrome refractories are desirable for many uses because they are substantially neutral in action when exposed to either acid or basic slags, and because chrome ore is relatively cheap and is one of the more refractory of the materials 20 commonly applied to such uses. Certain disadvantages, however, have militated against chrome refractories used prior to our invention. For instance, they have been characterized by relatively low softening temperatures; consequently, 25 their use has been limited to temperatures substantially below the melting point of chrome ore, and it has been necessary to restrict the loads applied to the refractories. Moreover, they have exhibited other properties undesirable in refractories for use at high temperatures, such as appreciable volume shrinkage upon reheating.

This invention is predicated on our discovery that its stated objects may be attained by making chrome refractories from mixtures of at 35 least 50 per cent of chrome ore with natural olivine in an amount not exceeding the chrome ore. Thus the refractories provided by the invention comprise from about 5 to not exceeding about 50 per cent of olivine and the balance substantially all chrome ore, and most advantageously they are composed of chrome ore with from about 20 to about 40 per cent of olivine.

The olivines used in the practice of the invention are of the Mg-Fe type. Preferably the olivine rock is high in its magnesium orthosilicate content, examples of suitable rocks being the dunites and peridotites. The iron content of the olivine should be relatively low, and most advantageously should not exceed about 10 per cent calculated as FeO. In the practice of the invention satisfactory results have been obtained with a dunite containing about 40.6 per cent of SiO<sub>2</sub>, 47.6 per cent of MgO, 7.5 per cent of FeO, 1.1 per cent of Al<sub>2</sub>O<sub>3</sub>, 0.8 per cent of Cr<sub>2</sub>O<sub>3</sub>, 0.1 per cent of CaO, and an ignition loss of 1.2 per

cent. The most highly serpentinized and most highly steatitized olivines are, in general, not suitable for the purposes of the present invention, nor other olivine minerals containing more than minor amounts of alteration products. However, we have successfully used olivines which contained as much as 10 to 15 per cent of talc-plus-serpentine, and depending upon the standards of refractoriness which the product must meet, it may be possible for some purposes to use olivine-rich materials containing somewhat greater percentages of these and other hydrous alteration products.

As exemplifying the benefits to be derived from the practice of the invention, reference may be made to refractories made from (a) a chrome ore containing about 32.7 per cent of Cr<sub>2</sub>O<sub>3</sub>, 14.5 per cent of FeO, 17.8 per cent of MgO, 29.5 per cent of Al<sub>2</sub>O<sub>3</sub>, and the balance consisting of other substances in small amounts, and (b) an olivine containing about 41 per cent of SiO<sub>2</sub>, 49 per cent of MgO, 7.7 per cent of iron calculated as FeO, 0.8 per cent of Al<sub>2</sub>O<sub>3</sub>, 0.4 per cent of CaO, 0.3 per cent of chromium calculated as Cr<sub>2</sub>O<sub>3</sub>, and an ignition loss of 0.8 per cent. A mixture of 15 per cent of that chrome ore and 25 per cent of olivine was ground to about 4 mesh and the ground mixture, after tempering with water, was formed into bricks and burned to about 2600° F. Brick for comparison were made in the same 20 manner from 100 per cent of the same chrome ore. Upon test the bricks showed the following 25 properties:

|                                                              | 75% chrome<br>ore—25%<br>olivine | 100%<br>chrome ore | 35 |
|--------------------------------------------------------------|----------------------------------|--------------------|----|
| Temperature of failure of brick under<br>load of 25#/sq. in. | 2700° F.                         | 2400° F.           | 40 |
| Volume change when reheated for 5<br>hours at 2912° F.       | -0.1%                            | -2.5%              |    |

It appears, therefore, that brick made in accordance with this invention possess a substantially higher temperature of failure, and that the volume change upon reheating has become practically nil, as compared with a high shrinkage upon reheating of ordinary chrome ore brick.

The foregoing results are characteristic of the properties achieved through the practice of this invention, indicating substantial increase in strength with great reduction, or virtual elimination, in shrinkage upon reheating. Although benefits are obtained by making refractories from chrome ore and more than about 5 per cent of

olivine, with the olivine not exceeding the amount of chrome ore, particularly desirable results are attained using mixtures of chrome ore and about 20 to 40 per cent of olivine because within this 5 range of compositions especially suitable combinations of properties are obtained. For instance, using 20 to 40 per cent of olivine the temperature of failure under load is increased materially as compared with brick made from chrome ore alone 10 in accordance with prior practice, and within this range the strongest mixes, as indicated by the moduli of rupture, are produced. Within this range also there is minimum change in linear dimensions in burning, so that the burning 15 shrinkage is very slight, as may be desirable in refractories. Moreover, these compositions show minimum change in linear dimensions upon re-heating, this change taking the form of shrinkage and being generally of the order of about 0.5 per 20 cent, and not exceeding about 2.0 per cent. Moreover, the porosity is relatively low for refractories of this type.

We have found also that the brick possess desirable weight characteristics. For instance, 25 those containing from about 20 to about 40 per cent of olivine exhibit weights from about 170 to 180 lbs. per cubic foot as compared with brick made from chrome ore alone, which may weigh as much as about 196 lbs. per cubic foot. This is 30 of importance because refractory brick of this type are commonly sold on a weight basis, and a reduction in weight thus means that the buyer obtains more brick per ton than with heavier brick, or, stated another way, the shipping cost 35 per brick is less because there are more brick per ton.

In the practice of the invention the chrome ore and olivine, suitably grain sized, are intimately mixed in accordance with desired practice. 40 The two materials may be ground together, or they may be ground separately. The particular grain size and relation of grain sizes of the two materials does not seem to be critical in achieving the benefits of the invention, but they may be 45 varied to vary properties, such as bulk density and porosity, of the resultant fired refractory in accordance with relations understood by those skilled in the art.

If the refractory is to be used as a lining or 50 ramming mix, or for similar purposes, it is necessary only to produce an intimate mixture of the two materials in appropriate proportions and suitably grain sized. Where shaped refractories are to be formed the materials are mixed in a 55 suitable mixer and tempered with water or other suitable liquid according to customary practice, for which reason mixing in an ordinary wet pan may be carried out. The prepared mixture is then shaped, advantageously under high pressure, and the bricks then dried and burned.

If the bricks are to be shipped unburned it will usually be desirable to add a temporary binder such as the organic binders and others which are well known and available in the art.

For some purposes it may be desirable also to 5 add a mineralizer such as borax, fluorspar, cryolite, and others of which a variety are used in the production of refractories. Usually the mineralizer will be present in rather small amount, usually not to exceed about 5 per cent.

In the practice of the invention a part or all of the chrome ore, alone or with olivine, may be calcined, if desired, prior to forming the batch, or if desired for any reason it may be fused and crushed to prepare it for the manufacture of the 15 refractories. Likewise, the chrome ore and the olivine, or either, may be subjected to the various purification and beneficiation treatments, such as magnetic separation, applied to removal of 20 impurities or to improve the quality of the mineral.

While the invention has been described chiefly with reference to the production of shaped and fired articles, nevertheless it contemplates also 25 the use of refractory compositions as ramming mixes, for forming linings, or the like, which are burned in place. Similarly, the brick may be formed and dried, shipped in that condition, and laid up into the desired structure, being burned in 30 service.

According to the provisions of the patent statutes, we have explained the principle and mode of applying our invention and have described what we now consider to represent its best embodiment. However, we desire to have 35 it understood that, within the scope of the appended claims, the invention may be practiced otherwise than as specifically described.

We claim:

1. A refractory material comprising about 5 40 to 50 per cent of olivine of high magnesium orthosilicate content, and the remainder substantially all chrome ore.

2. A burned refractory material comprising from about 5 to 50 per cent of olivine of high 45 magnesium orthosilicate content, and the remainder substantially all chrome ore.

3. A refractory material comprising from about 20 to 40 per cent of olivine of high magnesium orthosilicate content, and the remainder sub- 50 stantially all chrome ore.

4. A refractory material comprising about 75 per cent of chrome ore, and 25 per cent of olivine of high magnesium orthosilicate content.

5. A burned refractory material comprising 55 about 75 per cent of chrome ore, and 25 per cent of olivine of high magnesium orthosilicate content.

FREDERIC A. HARVEY.

RAYMOND E. BIRCH.

60